

## UNITED STATES PATENT OFFICE.

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MAINE.

## SHOE STIFFENER.

No Drawing.

Application filed December 21, 1922. Serial No. 608,358.

*To all whom it may concern:*

Be it known that I ALBERT L. CLAPP, a citizen of the United States, residing at Danvers, in the county of Essex and State 5 of Massachusetts, have invented new and useful Improvements in Shoe Stiffeners, of which the following is a specification.

This invention has for its object to produce a fibrous material containing a thermo- 10 plastic compound, for use as a shoe stiffener, such as a box toe or box-toe blank,—the more especial object being to provide a material of the class referred to which may be manufactured by the aid of the machinery 15 common to the manufacture of paper.

It has been almost the universal practice in the manufacture of such thermo-plastic or moldable box toes, first to form a fibrous sheet usually of wool or cotton and wool 20 felt, then to saturate or impregnate the sheet with a molten thermo-plastic compound or mixture, and, after the latter has cooled and set, to cut box-toe blanks of appropriate size and shape therefrom. A 25 box-toe blank thus formed has certain highly desirable characteristics flowing from the nature of the fibrous sheet. Since the sheet is a true felt, with numerous pores and interstices, it has the capacity for absorbing 30 and carrying a large amount, proportionate to its weight, of the thermo-plastic compound; and, because of the long fibers of 35 which it is composed, it may (when its contained thermo-plastic compound is fluxed or plastic) be stretched about the toe end of the last without danger of tearing. But the process of producing felt by the 40 usual or common felting machine is a long and expensive operation and the output is limited.

Any stiffened or moldable box-toe material must be capable of being stretched without tearing sufficiently to permit its being 45 drawn about the last in the pulling-over and end-lasting operations; that is, it must be possessed of a certain degree of tensile strength and yet must be capable of being stretched, and at the same time possess 50 toughness and durability.

After many experiments, I have succeeded 55 in producing from an aqueous pulp a box-toe material having the thermo-plastic compound incorporated therein and possessing the necessary qualities and characteristics hereinbefore referred to. This material,

which is sheeted on a common paper-making machine of the cylinder type (i. e. a wet machine), contains a very large percentage of the thermo-plastic stiffening compound, may be stretched and molded about the end 60 of the last without danger of being torn in the stretching operation, and possesses that stiffness and resiliency which is necessary to produce a successful box toe. The thermo-plastic compound is incorporated in 65 the pulp prior to the formation of the sheet, and one of the problems to be solved in accomplishing this result is to effect the retention of the thermo-plastic compound in the pulp. 70

The pulp must be made of those materials which will impart to the finished sheet the optimum characteristics hereinbefore referred to. I have found that it is possible to use cellulosic material or wood pulp 75 together with long hairs such as cattle hair or wool. It is recognized by paper manufacturers that the stock must be capable of being "formed" on the cylinder mold and built up on the make-up roll, and that it 80 must be of such character as will permit the incorporation of several times its weight of the thermo-plastic compound. The thermo-plastic compound must be of such character that it may be powdered or finely 85 reduced, that it should possess a relatively short melting-point-lag so that it will set rapidly when cooled after once being in molten condition, and that it should be capable of being softened upon the application 90 of moderate heat. As the thermo-plastic compound, I may use various bitumens, resins, gums and waxes in varying combinations. Thus I may use a mixture of say 60 parts of oil blown-asphalt having 95 a melting point say of 260° F., 30 parts of resin and 10 parts of montan wax, which are melted, thoroughly mixed, permitted to cool and harden, and then crushed or reduced to finely divided condition; or these 100 several ingredients may be mixed in proportions differing from those hereinbefore stated. On the other hand, I may employ as the thermo-plastic compound a blend or mixture of rosin, copal, montan or other 105 equivalent wax, drying oil and calcium resinate. All of these various materials, having the characteristics last referred to, are comprehended within the phrase "thermo-plastic compound." 110

The following example will serve to illustrate a box-toe material embodying the invention and the process of producing it. 5 parts of cellulosic material, such as sulphate or sulphite pulp or waste kraft or sulphite paper, together with 5 to 10 parts of tanned leather skivings, and 2 to 4 parts of caustic soda are placed in a common beating engine together with sufficient water to ensure the circulation of the stock, and are beaten until the leather has partially dissolved and the cellulose fibers have been more or less hydrated. While the leather is partly dissolved, a small quantity of gelatinous fibrous leather residuum remains. I now add to the beater about 5 parts of cattle hair (or wool), and, lifting the beater roll from the bed plate, I operate the beating engine until the hair is thoroughly mixed into the stock. It is desirable not to cut the hair into short pieces but to leave it in relatively long condition, preferably so that it retains its original length. I now add to the stock a large amount of the finely-divided thermo-plastic compound, say from 90 to 120 parts thereof, and the operation of the beater is continued until the thermo-plastic compound has been thoroughly distributed throughout the stock. In the particular example given, I ordinarily employ about 90 parts of a blend or mixture consisting of certain ingredients in the following proportions; namely, about 80% of acid resins of which about one-sixth is copal and the remainder rosin, about 15% montan wax, about 3% china wood oil, and about 2% of lime. These ingredients are thoroughly mixed together when molten and the lime reacts with certain acids of the resins to form a calcium resinate or soap.

After the thermo-plastic compound is thoroughly incorporated in and distributed throughout the pulp, I add about 20 parts of aluminum sulphate and the stock is further beaten until the alum is distributed throughout the pulp and has precipitated the dissolved leather in the form of a gelatinous hydrate which coagulates or precipitates and fixes upon the fibers the particles of thermo-plastic compound which are in the stock. The aqueous pulp is now transferred to a paper-making machine and formed into sheets of the desired caliper. Each sheet as stripped from the make-up roll is dried flat and then subjected to sufficient heat and pressure to melt the contained thermo-plastic compound and cause it to penetrate throughout and coalesce within the sheet. To accomplish this result, the sheet may be passed through calender rolls heated to the necessary temperature. The sheet is now cut into blanks of appropriate size and shape to serve as shoe stiffeners, such, for example, as box toes or counter stiffeners.

I may incorporate in the aqueous pulp

various other materials, such, for example, as red iron oxide or other coloring matter for imparting a desired color to the sheet material and/or to act as a filler. I may also incorporate in the pulp more or less of disintegrated box-toe waste or such material as wood flour.

The addition of the waste leather to the stock serves two purposes. That portion of the leather which is dissolved by caustic soda, when precipitated with alum or other precipitant, provides a coagulating medium for retaining the finely-divided thermo-plastic compound in the stock and fixing it upon the fibers so that only a relatively small proportion of the disintegrated thermo-plastic compound escapes with the white water. The fibrous leather residuum aids in forming the sheet on the wet machine and increases the strength of the resulting sheet. The presence of the long hairs in the stock permits the stock to be stretched and molded without being sheared or torn in the molding operation, whereas the cellulose fibers are necessary to give sufficient strength and "formation" to the sheet.

A box-toe blank, formed as herein described, possesses those characteristics and qualities which enable it to be successfully used in lieu of those heretofore produced, in which the felt is saturated with molten thermo-plastic compound, but may be produced in very large quantities and at relatively low expense. The fibrous materials which are utilized are of themselves inexpensive; namely, chemical wood pulp, cattle hair and other scrap. If sulphite or sulphate screenings be used, substantially all of the fibrous materials are of the nature of waste materials or by-products.

In the foregoing description it will be observed that the proportion of thermo-plastic compound to the cellulosic material and the hair is about 9 to 1 by weight, and, in fact, it may be even greater. In the finished product, the ratio of thermo-plastic compound to fibers is as 7.5 to 1,—a result which, so far as I know, has never before been achieved. Consequently the box toe when molded possesses, to a maximum degree, stiffness, toughness and resiliency, so that its shape is not easily distorted when incorporated in a shoe. The box-toe blank may be skived to present a sharp edge, which of itself is highly desirable in the manufacture of a high grade shoe.

What I claim is:—

1. A shoe stiffener adapted to be made limp and flexible upon the application of heat and comprising cellulose fibers, cattle hair, leather fibers, and thermo-plastic compound, with the fibers in felted relation and the thermo-plastic compound distributed throughout the fibers.

2. A shoe stiffener adapted to be made

flexible upon the application of heat and comprising cellulose fiber, long animal fibers and thermo-plastic compound, with the fibers in felted relation and the thermo-plastic compound distributed together with a precipitate throughout the fibers.

3. A shoe stiffener adapted to be made limp and flexible upon the application of heat and comprising cellulose fibers, cattle hair, leather fibers, and thermo-plastic compound, and a precipitate formed by the reaction of a precipitant with dissolved leather, the fibers being in felted relation and the thermo-plastic compound being distributed throughout the fibers.

4. A process of making shoe stiffeners, which comprises pulping cellulose fibers, leather in the presence of caustic soda, long fibers such as cattle hair, and a finely-divided thermo-plastic compound, then adding a precipitating agent for the dissolved leather, and sheeting the resultant pulp on a paper machine.

5. A process of making a shoe stiffener, which comprises beating together cellulose fiber, tanned leather and caustic soda in water, until the leather is more or less dissolved, incorporating long fibers and finely-divided or crushed thermo-plastic compound in the resulting pulp, adding a precipitating agent for reaction with the dissolved leather, and sheeting the pulpy mass on a paper machine.

6. A process of making a fibrous material suitable for shoe stiffeners, which comprises forming an aqueous fibrous pulp, incorporating a crushed thermo-plastic compound in the pulp, in the proportion of not less than six parts by weight of said compound to one part by weight of fibers, coagulating and fixing the thermo-plastic compound on the fibers, and sheeting the resulting pulp in a paper machine.

In testimony whereof I have affixed my signature.

ALBERT L. CLAPP.